



US005176976A

**United States Patent** [19]

Kikuchi et al.

[11] **Patent Number:** 5,176,976  
[45] **Date of Patent:** Jan. 5, 1993

[54] **ORGANIC ELECTRONIC MATERIAL AND ELECTROPHOTOGRAPHIC PHOTOSENSITIVE MEMBER CONTAINING SAME**

[75] Inventors: Toshihiro Kikuchi, Yokohama; Akio Maruyama, Kawasaki, both of Japan

[73] Assignee: Canon Kabushiki Kaisha, Tokyo, Japan

[21] Appl. No.: 680,824

[22] Filed: Apr. 5, 1991

[30] **Foreign Application Priority Data**

Apr. 9, 1990 [JP] Japan ..... 2-92183

[51] Int. Cl.<sup>5</sup> ..... G03G 5/047; G03G 5/09

[52] U.S. Cl. ..... 430/58; 430/70; 430/83; 355/211; 358/300; 552/304

[58] **Field of Search** ..... 430/58, 70, 83

[56] **References Cited**

**U.S. PATENT DOCUMENTS**

3,615,565 10/1971 Gerrach et al. ..... 430/495 X  
3,975,285 8/1976 Ohnishi et al. ..... 252/299  
4,222,902 9/1980 Hoffman et al. ..... 252/299  
4,728,592 3/1988 Ohaku et al. ..... 430/59

**FOREIGN PATENT DOCUMENTS**

52-04188 2/1977 Japan .  
54-58445 5/1979 Japan .  
54-151955 11/1979 Japan .  
55-52063 4/1980 Japan .  
55-42380 10/1980 Japan .  
58-19804 2/1983 Japan .

58-32372 7/1983 Japan .  
61-75355 4/1986 Japan .  
61-132955 6/1986 Japan .  
61-148159 7/1986 Japan .  
63-70257 3/1988 Japan .  
63-72664 4/1988 Japan .  
63-85749 4/1988 Japan .  
63-104061 5/1988 Japan .  
63-174993 7/1988 Japan .  
63-175860 7/1988 Japan .  
206349 8/1989 Japan ..... 430/70  
1183044 3/1970 United Kingdom .

*Primary Examiner*—Roland Martin  
*Attorney, Agent, or Firm*—Fitzpatrick, Cella, Harper & Scinto

[57] **ABSTRACT**

An organic electronic material comprises a compound represented by the following formula (I).



The compounds transport electrons and is excellent in durability when used in a photosensitive layer of an electrophotographic photosensitive member.

**10 Claims, 1 Drawing Sheet**



FIG. 1



FIG. 2

ORGANIC ELECTRONIC MATERIAL AND  
ELECTROPHOTOGRAPHIC PHOTOSENSITIVE  
MEMBER CONTAINING SAME

BACKGROUND OF THE INVENTION

1. Field of the Invention

The present invention relates to an organic electronic material, and an electrophotographic photosensitive member having superior electrophotographic performances attributable to the employment of the material.

2. Related Background Art

In recent years, function-separated electrophotographic photosensitive members, in which the function of generating charges and the function of transporting charges are shared by respectively separate electronic materials, have brought about a marked improvement in the sensitivity and durability properties for which conventional organic photosensitive members have been considered to have disadvantages.

Such function-separated electrophotographic photosensitive members allow a wide range of selection of materials for charge-generating materials and charge-transporting materials, and hence can also be advantageous in, e.g., that electrophotographic photosensitive members having the desired performance can be produced with a greater ease and at a low cost.

As the charge-generating materials, various materials are known, including azo pigments, polycyclic quinone pigments, cyanine dyes, squaric acid dyes and pyrylium salt dyes.

Of these, azo pigments have the advantages that they have a high light-fastness, have a high charge-generating ability and can be synthesized with ease. Hence, many materials have been proposed.

As for the charge-transporting materials, known materials are exemplified by the pyrazolone compounds as disclosed in Japanese Patent Publication No. 52-4188, the hydrazone compounds as disclosed in Japanese Patent publication No. 55-42380 and Japanese Patent Application Laid-open No. 55-52063, the triphenylamine compounds as disclosed in Japanese Patent Publication No. 58-32372 and Japanese Patent Application Laid-open No. 61-132955, and the stilbene compounds as disclosed in Japanese Patent Applications Laid-open No. 54-151955 and No. 58-19804.

However, almost all of the known charge-transporting materials noted in the above, in particular, the charge-transporting materials used in organic electrophotographic photosensitive members practically used, have the properties of transporting positive holes.

When a charge-transporting material capable of transporting positive holes is used in an electrophotographic photosensitive member comprising a conductive support and, provided thereon, a charge generation layer and a charge transport layer in this order, i.e. having the conventional structure most commonly used, the polarity of the primary charge to the photosensitive member is negative. When the photosensitive member is negatively charged, ozone is generated. This ozone has a bad chemical influence on photosensitive members.

Now, as a countermeasure to the deterioration of photosensitive members due to the ozone generated in negative charging, a proposal has been made in, for example, Japanese Patent Applications Laid-open No. 61-753555 and No. 54-58445 on an electrophotographic photosensitive member comprising a support and, pro-

vided thereon, a charge transport layer and a charge generation layer in this order.

Since, however, in the electrophotographic photosensitive member with such layer constitution, the relatively thin charge generation layer is provided as an upper layer, a serious deterioration of performance is caused by the wear that accompanies repeated use.

When a photosensitive member is provided with a protective layer made of an organic insulating material for the purpose of preventing such wear, it has been impossible to maintain stable performances because of unstable potential after repeated use.

Under such circumstances, it has been sought to develop an organic electronic material capable of transporting electrons. Conventionally proposed charge-transporting materials capable of transporting electrons include, for example, 2,4,7-trinitro-9-fluorenone (TNF), the dicyanomethylenefluorene carboxylates as disclosed in Japanese Patent Application Laid-open No.

15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980

tive support and a photosensitive layer provided on the conductive support; the photosensitive layer contains a compound represented by the following formula (I).



Formula (I)

5

10

15

wherein R<sub>1</sub>, R<sub>2</sub>, R<sub>3</sub> and R<sub>4</sub> each represents a hydrogen atom, an alkyl group, an aralkyl group or an aryl group, and R<sub>1</sub>, R<sub>2</sub>, R<sub>3</sub> and R<sub>4</sub> may be the same or different one another.

20

#### BRIEF DESCRIPTION OF THE DRAWINGS

FIG. 1 schematically illustrates an example of the constitution of an electrophotographic apparatus in which the electrophotographic photosensitive member of the present invention is used.

FIG. 2 is a block diagram of a facsimile system in which the electrophotographic photosensitive member of the present invention is used.

30

#### DESCRIPTION OF THE PREFERRED EMBODIMENTS

The present invention is an organic electronic material containing a compound represented by the following formula (I), and an electrophotographic photosensitive member having a photosensitive layer containing such a compound.

40



Formula (I)

45

50

wherein R<sub>1</sub>, R<sub>2</sub>, R<sub>3</sub> and R<sub>4</sub> each represents a hydrogen atom, an alkyl group, an aralkyl group or an aryl group, and R<sub>1</sub>, R<sub>2</sub>, R<sub>3</sub> and R<sub>4</sub> may be the same or different.

55

In the formula (I), the alkyl group may include groups such as methyl, ethyl, n-propyl, n-butyl and t-butyl. The aralkyl group may include groups such as benzyl and phenethyl. The aryl group may include groups such as phenyl and naphthyl.

60

Typical examples of the stilbenequinone compounds represented by the formula (I) are shown below. The compounds are by no means limited to these.

65

The examples of the compound are set forth by showing the substituents R<sub>1</sub>, R<sub>2</sub>, R<sub>3</sub> and R<sub>4</sub> variable in the following base structure.



Exemplary Compound (1)

R<sub>1</sub>, R<sub>2</sub>, R<sub>3</sub>, R<sub>4</sub>: -CH<sub>3</sub>

Exemplary Compound (2)

R<sub>1</sub>, R<sub>2</sub>, R<sub>3</sub>, R<sub>4</sub>: -H

Exemplary Compound (3)

R<sub>1</sub>, R<sub>2</sub>, R<sub>3</sub>, R<sub>4</sub>: -C<sub>2</sub>H<sub>5</sub>

Exemplary Compound (4)

R<sub>1</sub>, R<sub>2</sub>, R<sub>3</sub>, R<sub>4</sub>: -t-C<sub>4</sub>H<sub>9</sub>

Exemplary Compound (5)

R<sub>1</sub>, R<sub>2</sub>: -CH<sub>3</sub>R<sub>3</sub>, R<sub>4</sub>: -t-C<sub>4</sub>H<sub>9</sub>

Exemplary Compound (6)

R<sub>1</sub>, R<sub>2</sub>: -C<sub>2</sub>H<sub>5</sub>R<sub>3</sub>, R<sub>4</sub>: -n-C<sub>4</sub>H<sub>9</sub>

Exemplary Compound (7)

R<sub>1</sub>, R<sub>2</sub>: HR<sub>3</sub>, R<sub>4</sub>: -n-C<sub>4</sub>H<sub>9</sub>

Exemplary Compound (8)

R<sub>1</sub>: -CH<sub>3</sub>; R<sub>2</sub>: -C<sub>2</sub>H<sub>5</sub>R<sub>3</sub>: -CH<sub>3</sub>; R<sub>4</sub>: -C<sub>2</sub>H<sub>5</sub>

Exemplary Compound (9)

R<sub>1</sub>: -CH<sub>3</sub>; R<sub>2</sub>: -C<sub>2</sub>H<sub>5</sub>R<sub>3</sub>: -C<sub>2</sub>H<sub>5</sub>; R<sub>4</sub>: -CH<sub>3</sub>

Exemplary Compound (10)

R<sub>1</sub>, R<sub>2</sub>: -CH<sub>3</sub>

Exemplary Compound (11)

R<sub>1</sub>, R<sub>2</sub>: -n-C<sub>3</sub>H<sub>7</sub>R<sub>3</sub>, R<sub>4</sub>: -t-C<sub>4</sub>H<sub>9</sub>

Exemplary Compound (12)



Exemplary Compound (13)



Exemplary Compound (14)





Exemplary Compound (15)  
R<sub>1</sub>, R<sub>2</sub>: -n-C<sub>3</sub>H<sub>7</sub>



Exemplary Compound (16)



The organic electronic material of the present invention can be used in, for example, the photosensitive layer of the electrophotographic photosensitive member.

The electrophotographic photosensitive member can be constituted in any of the following forms:

- (1) On a conductive support, a layer containing a charge-generating material and a layer containing a charge-transporting material are successively laminated.
- (2) On a conductive support, a layer containing a charge-transporting material and a layer containing a charge-generating material are successively laminated.
- (3) On a conductive support, a layer containing a charge-generating material and a charge-transporting material is formed.
- (4) On a conductive support, a layer containing a charge-transporting material and a layer containing a charge-generating material and a charge-transporting material are successively laminated.
- (5) On a conductive support, a layer containing a charge-generating material and a layer containing a charge-generating material and a charge-transporting material are successively laminated.

The stilbenequinone compound represented by the formula (I) of the present invention is so highly capable of transporting electrons that it can be used as the charge-transporting material in the photosensitive layer of the electrophotographic photosensitive member of any of the above forms. In the case when the electrophotographic photosensitive member is of form (1), it can be preferably used in positive charging, and in the case of form (2), in negative charging. In the cases of forms (3), (4) and (5), the photosensitive members can be used in any of positive charging and negative charging.

In the present invention, the form (1) is particularly preferred among the above embodiments. However, the embodiments the electrophotographic photosensitive

member in the present invention are by no means limited to the above.

The constitution of the present invention will be further detailed below.

5 The charge-generating material used in the present invention may be any of those capable of generating charges as charge-generating materials. It may include, for example, the following:

- (1) Azo pigments such as monoazo, bisazo and trisazo pigments.
- (2) Phthalocyanine pigments such as metal phthalocyanine and metal-free phthalocyanine.
- (3) Indigo pigments such as indigo and thioindigo.
- (4) Perylene pigments such as perylene anhydrides and perylene imides.
- (5) Polycyclic quinone pigments such as anthraquinone and pyrenequinone.
- (6) Squarilium dyes.
- (7) Pyrylium salts and thiopyrylium salts.
- (8) Triphenylmethane dyes.
- (9) Inorganic materials such as selenium and amorphous silicon.

These charge-generating material may be used alone or in combination of two or more kinds.

25 The layer that contains the charge-generating material, i.e., the charge generation layer can be formed by dispersing the charge-generating material as described above in a suitable binder and by coating a conductive support with the dispersion. It can also be formed by forming a thin film or by a dry process such as sputtering or CVD.

30 The binder can be selected from a vast range of binder resins including, for example, polycarbonate, polyester, polyacrylate, butyral resins, polystyrene, polyvinyl acetal, diallylphthalate resins, acrylic resins, methacrylic resins, vinyl acetate resins, phenol resins, silicone resins, polysulfone, a styrene-butadiene copolymer, alkyd resins, epoxy resins, urea resins and a vinyl chloride-vinyl acetate copolymer. The binder is by no means limited to these.

35 These resins may be used alone, in the form of a copolymer of any of these components or in the form of a mixture of two or more kinds of resins.

40 The resin amount contained in the charge generation layer is preferably in an amount of not more than 80% by weight, and particularly preferably not more than 40% by weight, based on the total weight of the layer.

45 The charge generation layer may preferably have a layer thickness of not more than 5  $\mu\text{m}$ , and particularly from 0.01  $\mu\text{m}$  to 2  $\mu\text{m}$ .

50 Various sensitizers may be further added to the charge generation layer.

55 The layer that contains the charge-transporting material, i.e., the charge transport layer can be formed by combination of the stilbenequinone compound represented by the formula (I) with a suitable binder resin.

In the present invention, a charge-transporting material of a different type can also be used in combination.

60 The binder resin used may include, in addition to those used in the charge generation layer, photoconductive polymers such as polyvinyl carbazole and polyvinyl anthracene.

65 As to the mixing proportion of this binder resin to the stilbenequinone compound represented by the formula (I), the stilbenequinone compound may preferably be in an amount of from 10 parts by weight to 500 parts by weight based on 100 parts by weight of the binder.

The charge transport layer may preferably have a layer-thickness of from 5  $\mu\text{m}$  to 40  $\mu\text{m}$ , and particularly from 10  $\mu\text{m}$  to 30  $\mu\text{m}$ .

It is also possible to optionally further add in the charge transport layer an antioxidant, an ultraviolet absorbent, a plasticizer or a conventionally known charge-transporting material.

When the photosensitive layer is constituted according to the form (3), i.e., when it is a single-layer structure, a coating solution prepared by dispersing or dissolving the charge-generating material previously described and the compound represented by the formula (I) in a suitable binder above mentioned may be applied to a support to form a layer. This layer may preferably have a thickness of from 5  $\mu\text{m}$  to 40  $\mu\text{m}$ , and particularly preferably from 10  $\mu\text{m}$  to 30  $\mu\text{m}$ .

In the present invention, a layer having a barrier function and an adhesive function, i.e., a subbing layer, can also be provided between the conductive support and the photosensitive layer.

Materials for the subbing layer may include polyvinyl alcohol, polyethylene oxide, ethyl cellulose, methyl cellulose, casein, polyamide, glue and gelatin.

These materials may be dissolved in a suitable solvent and the resulting solution may be coated on the conductive support. The subbing layer thus formed may preferably have a coating thickness of not more than 5  $\mu\text{m}$ , and particularly from 0.2 to 3.0  $\mu\text{m}$ .

In the present invention, a resin layer or a resin layer in which a conductive material has been dispersed may also be provided on the photosensitive layer so that the photosensitive layer can be protected from mechanical and electrical external forces.

All the layers described above can be formed on the conductive support by any coating processes such as dip coating, spray coating, spin coating, roller coating, Meyer bar coating and blade coating, using a suitable organic solvent.

The conductive support in the present invention may include, for example, supports of the following forms:

- (1) A support comprising a metal such as aluminum, an aluminum alloy, stainless steel or copper, formed into a plate or a drum.
- (2) A support comprising a non-conductive support made of glass, resin or paper, or the above conductive support (1), on which a film has been formed by vacuum deposition of a metal such as palladium, rhodium, gold or platinum or by lamination of a film of such a metal.
- (3) A support comprising a non-conductive support made of glass, resin or paper, or the above conductive support (1), on which a layer comprised of a conductive compound such as a conductive polymer, tin oxide or indium oxide has been formed by vacuum deposition or coating.

The electrophotographic photosensitive member of the present invention can be applied not only in electrophotographic copying machines, but also facsimile machines, laser printers, CRT printers. It can also be widely used in electrophotographic lithography systems and so forth in which electrophotography is applied.

FIG. 1 schematically illustrates an example of the constitution of a transfer electrophotographic apparatus in which the electrophotographic photosensitive member according to the present invention is used.

As shown in FIG. 1, the numeral 1 denotes a drum photosensitive member serving as an image supporting

member, which is rotated around a shaft 1a at a given peripheral speed in the direction shown by arrow. In the course of rotation, the photosensitive member 1 is uniformly charged on its periphery, with positive or negative given potential by the operation of a charging means 2, and then photoimaginewise exposed to light L (slit exposure, laser beam scanning exposure, etc.) at an exposure zone 3 by the operation of an imagewise exposure means (not shown). As a result, electrostatic latent images corresponding to the exposure images are successively formed on the periphery of the photosensitive member.

The electrostatic latent images thus formed are subsequently developed by toner by the operation of a developing means 4. The resulting toner-developed images are then successively transferred by the operation of a transfer means 5, to the surface of a transfer medium P fed from a paper feed section (not shown) to the part between the photosensitive member 1 and the transfer means 5 in the manner synchronized with the rotation of the photosensitive member 1.

The transfer medium P on which the images have been transferred is separated from the surface of the photosensitive member and led through an image-fixing means 8, where the images are fixed and then delivered to the outside as a transcript (a copy).

The surface of the photosensitive member 1 after the transfer of images is cleaned of excess toner remaining after the transfer, using a cleaning means 6. Thus the photosensitive member is cleaned on its surface, further subjected to charge elimination by a pre-exposure means 7, and then repeatedly used for the formation of images.

The charging means 2 for providing uniform charge on the photosensitive member 1 include corona chargers, which are widely used. As the transfer means 5, corona transfer units are also widely used.

The electrophotographic apparatus may comprise a combination of plural components selected from the constituents such as the above photosensitive member, developing means and cleaning means and joined as one device unit so that the unit can be freely mounted on or detached from the body of the apparatus. For example, at least one of the charging means, developing means and cleaning means is joined with the photosensitive member into one device unit so that the unit can be freely mounted or detached using a guide means such as a rail provided in the body of the apparatus.

When the electrophotographic apparatus is used for a copying machine or a printer, the optical image exposing light L is the light reflected from, or transmitted through an original. Alternatively, L is the scanning laser beam or the light derived by driving an LED array or a liquid crystal shutter array, both according to signals obtained by reading an original with a sensor and converting the information into signals.

When used as a printer of a facsimile machine, the optical image exposing light L serves as exposing light used for the printing of received data. FIG. 2 illustrates an example thereof in the form of a block diagram.

As shown in FIG. 2, a controller 11 controls an image reading part 10 and a printer 19. The whole of the controller 11 is controlled by CPU 17. Image data output from the image reading part is sent to the other facsimile station through a transmitting circuit 13. Data received from the other station is sent to a printer 19 through a receiving circuit 12. Given image data are stored in an

image memory 16. A printer controller 18 controls the printer 19. The numeral 14 denotes a telephone.

An image received from a circuit 15 (image information from a remote terminal connected through the circuit) is demodulated in the receiving circuit 12, and then successively stored in an image memory 16 after the image information is decoded by the CPU 17. Then, when images for at least one page have been stored in the memory 16, the image recording for that page is carried out. The CPU 17 reads out the image information for one page from the memory 16 and sends the coded image information for one page to the printer controller 18. The printer controller 18, having received the image information for one page from the CPU 17, controls the printer 19 so that the image information for one page is recorded.

The CPU 17 receives image information for next page in the course of the recording by the printer 19.

Images are received and recorded in the above way.

#### EXAMPLE 1

To 600 ml of an aqueous solution consisting of 5.5 g (138 mmol) of sodium hydroxide and 66 g (200 mmol) of potassium hexacyanoferrate, 200 ml of an ethanol solution containing 4.50 g (33 mmol) of 2,4,6-trimethylphenol and 7.27 g (33 mmol) of 2,6-di-t-butyl-4-methylphenol, were dropwise added in 20 minutes with stirring. After the stirring was continued for five hours, precipitated crystals were collected. The resulting crude crystals were purified by silica gel column chromatography to give 2.1 g of a compound of the exemplary compound (5) (Yield: 18%).

Results of elementary analysis of this compound are shown below.

|             | C      | H     |
|-------------|--------|-------|
| Calculated: | 82.24% | 8.63% |
| Found:      | 82.19% | 8.69% |

Characteristics of the resulting compound were evaluated in the following manner.

First, 4 g of oxytitanium phthalocyanine obtained according to a preparation example disclosed in Japanese Patent Application Laid-open No. 61-239248 (U.S. Pat. No. 4,728,592) was added to a solution prepared by dissolving 7 g of polyvinyl butyral (degree of butyralation: 68 mol %; weight average molecular weight: 35,000) in 95 ml of cyclohexanone, and these were dispersed together for 20 hours using a sand mill. A coating solution was thus prepared.

This coating solution was diluted and thereafter applied to an aluminum sheet by Meyer bar coating so as

35

to give a dried coating thickness of 0.1  $\mu\text{m}$ . A charge generation layer was thus formed.

Next, 5 g of the compound obtained as above mentioned as a charge-transporting material and 6 g of polycarbonate (weight average molecular weight: 35,000) were dissolved in 100 g of chlorobenzene, and the resulting solution was coated on the charge generation layer by Meyer bar coating, followed by drying to form a charge transport layer with a dried coating thickness of 14  $\mu\text{m}$ . Thus an electrophotographic photosensitive member was obtained.

This electrophotographic photosensitive member was corona-charged by a static system at +6 kV using an electrostatic copy paper test machine (Model EPA-8100, manufactured by Kawaguchi Denki K. K.). The charged member was maintained in dark for 1 second, followed by exposure to light with illuminance of 20 lux to examine their charge characteristics.

Measured as the charge characteristics were the surface potential ( $V_0$ ), the potential ( $V_1$ ) after the dark-decaying for 1 second and the quantity of exposure ( $E_1$ ) required for reducing the potential ( $V_1$ ) to  $\frac{1}{2}$  the original value.

To also evaluate potential stability after repeated use, 25 the electrophotographic photosensitive member produced in the above was mounted on a cylinder for a photosensitive drum of a modified copying machine (NP-6650, manufactured by Canon Inc). After copies were taken on 2,000 sheets using this copying machine, the dark-portion potential ( $V_D$ ) and light-portion potential ( $V_L$ ) were measured. Initial  $V_D$  and  $V_L$  were set to be +650 V and +150 V, respectively.

Results obtained are shown in Table 1.

#### EXAMPLES 2 TO 7

Compounds of the exemplary compounds (1), (4), (6), (13) and (15) were obtained in the same manner as in Example 1 except that the 2,4,6-trimethylphenol and 2,6-di-t-butyl-4-methylphenol used in Example 1 were replaced with i) 2,4,6-trimethylphenol alone, ii) 2,6-di-t-butyl-4-methylphenol alone, iii) 2,6-dimethyl-4-methylphenol and 2,6-di-n-butyl-4-methylphenol, iv) 2,4,6-trimethylphenol and 2-benzyl-4,6-dimethylphenol, v) 4,6-dimethyl-2-phenylphenol alone and vi) 4-methyl-2,6-di-n-propylmethylphenol and 4-methyl-2,6-diphenylphenol, respectively.

Electrophotographic photosensitive members were prepared in the same manner as in Example 1 except for use of the respective compounds, and evaluation was made similarly.

Results obtained are shown in Table 1.

TABLE 1

| Exemplary compound | $V_0$<br>(+V) | $V_1$<br>(+V) | $E_1$<br>(lux · sec) | Initial stage |               | After 2,000 sheet running |               |
|--------------------|---------------|---------------|----------------------|---------------|---------------|---------------------------|---------------|
|                    |               |               |                      | $V_D$<br>(+V) | $V_L$<br>(+V) | $V_D$<br>(+V)             | $V_L$<br>(+V) |
| <u>Example:</u>    |               |               |                      |               |               |                           |               |
| 1                  | (5)           | 690           | 685                  | 2.8           | 650           | 150                       | 649           |
| 2                  | (1)           | 698           | 690                  | 2.9           | 650           | 150                       | 641           |
| 3                  | (4)           | 700           | 695                  | 3.0           | 650           | 150                       | 645           |
| 4                  | (6)           | 701           | 697                  | 2.0           | 650           | 150                       | 650           |
| 5                  | (10)          | 697           | 694                  | 2.5           | 650           | 150                       | 642           |
| 6                  | (13)          | 694           | 690                  | 2.4           | 650           | 150                       | 647           |
| 7                  | (15)          | 690           | 685                  | 2.0           | 650           | 150                       | 640           |

## COMPARATIVE EXAMPLES 1 TO 4

Electrophotographic photosensitive members were prepared in the same manner as in Example 1 except for

-continued  
Laid-open No. 63-85749)

Results obtained are shown in Table 2.

TABLE 2

| Comparative compound       | V <sub>0</sub><br>(+ V) | V <sub>1</sub><br>(+ V) | E <sub>I</sub><br>(lux · sec) | Initial stage           |                         | After 2,000 sheet running |                         |
|----------------------------|-------------------------|-------------------------|-------------------------------|-------------------------|-------------------------|---------------------------|-------------------------|
|                            |                         |                         |                               | V <sub>D</sub><br>(+ V) | V <sub>L</sub><br>(+ V) | V <sub>D</sub><br>(+ V)   | V <sub>L</sub><br>(+ V) |
| <u>Comparative Example</u> |                         |                         |                               |                         |                         |                           |                         |
| 1                          | (1)                     | 690                     | 671                           | 5.9                     | 650                     | 150                       | 601                     |
| 2                          | (2)                     | 691                     | 680                           | 84.0                    | —*                      | —*                        | —*                      |
| 3                          | (3)                     | 692                     | 687                           | 7.5                     | —*                      | —*                        | —*                      |
| 4                          | (4)                     | 711                     | 704                           | 14.5                    | —*                      | —*                        | —*                      |

\*Comparative Examples 2 to 4 showed such poor sensitivities and such high residual potentials that it was impossible to set potentials.

use of the following comparative compounds as charge- 20 transporting materials. Evaluation was also made similarly.



A compound of the exemplary compound (3) was obtained in the same manner as in Example except that the 2,4,6-trimethylphenol and 2,6-di-t-butyl-4-methylphenol were replaced with 2,4,6-triethylphenol.

Characteristics of the resulting compound were evaluated in the following manner.

On an aluminum substrate, a solution prepared by dissolving 5 g of N-methoxymethylated nylon 6 resin (weight average molecular weight: 32,000) and 5 g of alcohol soluble copolymer nylon (weight average molecular weight: 29,000) in 95 g of methanol was applied by Meyer coating to form a subbing layer with a dried coating thickness of 1  $\mu$ m.

Next, 1 g of a charge-generating material of the following structural formula:



0.6 g of polyvinyl butyral (degree of butyralation: 70%; weight average molecular weight: 50,000) and 60 g of dioxane were dispersed for 20 hours using a ball mill.

The resulting dispersion was applied by blade coating on the subbing layer already formed, to form a charge generation layer with a dried coating thickness of 0.1  $\mu\text{m}$ .

Next, 10 g of a compound of the exemplary compound (3) previously obtained and 10 g of polymethyl methacrylate (weight average molecular weight: 50,000) were dissolved in 110 g of chlorobenzene, and the resulting solution was applied by blade coating on the charge generation layer already formed, to form a charge transport layer with a dried coating thickness of 13  $\mu\text{m}$ .

An electrophotographic photosensitive member thus produced was corona-charged at +6 kV. The surface potential ( $V_0$ ) at this time was measured. The surface potential ( $V_1$ ) after this photosensitive member was left in the dark for 1 second was also measured. The sensitivity was evaluated based on the measurement of the quantity of exposure ( $E_1$ :  $\mu\text{J}/\text{cm}^2$ ) required for reducing the potential  $V_1$  after the dark-decaying to one-half. Here, a gallium-aluminum-arsenic three-component semiconductor laser (output: 5 mW; oscillation wavelength: 780 nm) was used as a light source.

Results obtained are shown below:

$V_0$ : +682 V

$V_1$ : +671 V

$E_1$ : 2.1  $\mu\text{J}/\text{cm}^2$

Next, the above photosensitive member was fitted to a modified machine of a transfer development type digital copier NP-9330, manufactured by Canon Inc., equipped with the same semiconductor laser as the above, to carry out an actual image forming test.

The test was carried out under the surface potential after primary charging and the surface potential after exposure set to +600 V and +100V, respectively (quantity of exposure: 2.0  $\mu\text{J}/\text{cm}^2$ ). Both characters and pictures were printed in a good state.

Images were further continuously produced on 3,000 sheets. As a result, stable prints were obtained from the initial stage to 3,000th sheet printing.

#### EXAMPLE 9

First, 7 g of oxytitanium phthalocyanine obtained according to a preparation example disclosed in Japanese Patent Application Laid-open No. 62-67094 (U.S. Pat. No. 4,664,997) was added to a solution prepared by dissolving 4 g of polyvinyl benzal (degree of benzalation: 78 mol %; weight average molecular weight: 100,000) in 100 g of cyclohexanone, and was dispersed for 48 hours using a ball mill. The resulting dispersion was applied on an aluminum sheet by Meyer bar coating, followed by drying at 90° C. for 30 minutes to form a charge generation layer with a thickness of 0.15  $\mu\text{m}$ .

Next, a solution prepared by dissolving 5 g of a compound of the exemplary compound (5) obtained in the same manner as in Example 1 and 5 g of a bisphenol Z polycarbonate resin (weight average molecular weight: 50,000) in 70 g of a mixed solvent of chlorobenzene/N,N-dimethylformamide (1 part by weight/1 part by weight) was applied by Meyer bar coating on the charge generation layer already formed, followed by drying at 130° C. for 2 hours to form a charge transport layer with a thickness of 18  $\mu\text{m}$ .

Charge characteristics of the electrophotographic photosensitive member thus prepared was evaluated in the same manner as in Example 8 to obtain the following results:

$V_0$ : +690 V

$V_1$ : +685 V

$E_1$ : 2.0  $\mu\text{J}/\text{cm}^2$

#### EXAMPLE 10

A compound of the exemplary compound (8) was obtained in the same manner as in Example 1 except that the 2,4,6-trimethylphenol and 2,6-di-t-butyl-4-methylphenol were replaced with 2-ethyl-4,6-dimethylphenol.

Characteristics of the resulting compound were evaluated in the following manner.

Two grams of a dye represented by the following structural formula:



and 4 g of the compound of the exemplary compound (8) were mixed in 40 g of a toluene (70 parts by weight)/N,N-dimethylformamide (30 parts by weight) solution of polycarbonate (weight average molecular weight: 30,000), and then dispersed for 10 hours using a ball mill. The resulting dispersion was diluted and thereafter applied on an aluminum sheet by Meyer bar coating, followed by drying at 100° C. for 1.6 hours to form a photosensitive layer with a thickness of 14  $\mu\text{m}$ .

Electrophotographic performance of the electrophotographic photosensitive member thus prepared was evaluated in the same manner as in Example 1. Results obtained are shown below:

$V_0$ : +685 V

$V_1$ : +685 V

$E_1$ : 3.6 lux.sec

Initial potential:

$V_D$ : +650 V

$V_L$ : +150 V

Potential after 10,000 sheet running:

$V_D$ : +639 V

$V_L$ : +161 V

#### EXAMPLE 11

A compound of the exemplary compound (11) was obtained in the same manner as in Example 1 except that the 2,4,6-trimethylphenol and 2,6-di-t-butyl-4-methylphenol were replaced with 4-methyl-2,6-di-n-propylphenol and 2,6-di-t-butyl-4-methylphenol.

Characteristics of the resulting compound were evaluated in the following manner.

On an aluminum substrate, a methanol solution of 5% of alcohol-soluble copolymer nylon (weight average molecular weight: 80,000) was applied to form a subbing layer with a dried coating thickness of 1  $\mu\text{m}$ .

Next, as a charge-generating material, 5 g of a trisazo pigment of the following structural formula:



was dispersed in 50 ml of tetrahydrofuran, using a sand mill.

Subsequently, 5 g of the compound of the exemplary compound (11) and 10 g of polycarbonate (weight average molecular weight: 35,000) were dissolved in a mixed solvent of chlorobenzene (70 parts by weight) and dichloromethane (30 parts by weight), and the resulting solution was added to the dispersion previously prepared, followed by further dispersion for 10 hours using a sand mill.

The resulting dispersion was applied by Meyer bar coating on the subbing layer already formed, so as to give a dried coating thickness of 16  $\mu\text{m}$ .

Charge characteristics of the electrophotographic photosensitive member thus prepared was measured in the same manner as in Example 1 to obtain the following results:

$V_0: +685 \text{ V}$   
 $V_1: +680 \text{ V}$   
 $E_t: 4.0 \text{ lux.sec}$

#### EXAMPLE 12

In 70 g of chlorobenzene, 5 g of a compound of the exemplary compound (6) obtained in the same manner as in Example 4 as a charge-transporting material and 5 g of polycarbonate (weight average molecular weight: 35,000) were dissolved to give a solution. This solution was applied on an aluminum sheet by Meyer bar coating to form a charge transport layer with a dried coating thickness of 14  $\mu\text{m}$ .

Next, 2 g of disazo pigment represented by the following structural formula:



was added to a solution prepared by dissolving 1 g of polyvinyl butyral (degree of butyralation: 80 mol %) 1 g dissolved in 45 ml of cyclohexanone, and these were

dispersed together for 24 hours using a sand mill. A coating dispersion was thus prepared.

This coating dispersion was diluted and thereafter applied to the above charge transport layer by Meyer bar coating so as to give a dried coating thickness of 0.3  $\mu\text{m}$ . A charge generation layer was thus formed. Using this charge generation layer, an electrophotographic photosensitive member was obtained.

Charge characteristics of this electrophotographic photosensitive member were evaluated in the same manner as in Example 1 except that the corona-charging was carried out at -5 kV.

Results obtained are shown below.

$V_0: -680 \text{ V}$   
 $V_1: -665 \text{ V}$   
 $E_t: 3.5 \text{ lux.sec}$

We claim:

1. An electrophotographic photosensitive member comprising a conductive support and a photosensitive layer provided on said conductive support; said photosensitive layer containing a compound having electron transporting properties represented by the following formula (I).



Formula (I)

wherein R1, R2, R3 and R4 each represents a hydrogen atom, an alkyl group, an aralkyl group or an aryl group, and R1, R2, R3 and R4 may be the same or different.

2. An electrophotographic photosensitive member according to claim 1, wherein said photosensitive layer comprises a charge generation layer and a charge transport layer.

3. An electrophotographic photosensitive member according to claim 2, wherein said charge transport layer is laminated on said charge generation layer.

4. An electrophotographic photosensitive member according to claim 2, wherein said charge generation layer is laminated on said charge transport layer.

5. An electrophotographic photosensitive member according to claim 1, wherein said photosensitive layer has a single-layer structure.

6. An electrophotographic photosensitive member according to claim 1, wherein a subbing layer is provided between said conductive support and said photosensitive layer.

7. An electrophotographic photosensitive member according to claim 1, wherein a protective layer is provided on said photosensitive layer.

8. An electrophotographic apparatus comprising an electrophotographic photosensitive member, an electrostatic latent image forming means, a means for developing the electrostatic latent image formed, and a means for transferring the developed image to a transfer medium;

said electrophotographic photosensitive member comprising a conductive support and a photosensitive layer provided on said conductive support; said photosensitive layer containing a compound having electron transporting properties represented by the following formula (I).



35 Formula (I)

wherein R<sub>1</sub>, R<sub>2</sub>, R<sub>3</sub> and R<sub>4</sub> each represents a hydrogen atom, an alkyl group, an aralkyl group or an aryl group, and R<sub>1</sub>, R<sub>2</sub>, R<sub>3</sub> and R<sub>4</sub> may be the same or different.

9. A device unit comprising an electrophotographic photosensitive member, a CHARGING means, DEVELOPING and a cleaning means;

50

said electrophotographic photosensitive member comprising a conductive support and a photosensitive layer provided on said conductive support; said photosensitive layer containing a compound having electron transporting properties represented following formula (I).



Formula (I)

wherein R<sub>1</sub>, R<sub>2</sub>, R<sub>3</sub> and R<sub>4</sub> each represents a hydrogen atom, an alkyl group, an aralkyl group or an aryl group, and R<sub>1</sub>, R<sub>2</sub>, R<sub>3</sub> and R<sub>4</sub> may be the same or different; and said device unit holding said electrophotographic photosensitive member, developing means and cleaning means as one unit, and said device unit being detachably provided in the body of an electrophotographic apparatus.

10. A facsimile machine comprising an electrophotographic apparatus and a receiver means for receiving image information from a remote terminal:

said electrophotographic apparatus comprising an electrophotographic photosensitive member; and said electrophotographic photosensitive member comprising a conductive support and a photosensitive layer provided on said conductive support; said photosensitive layer containing a compound having electron transporting properties represented by the following formula (I).



Formula (I)

wherein R<sub>1</sub>, R<sub>2</sub>, R<sub>3</sub> and R<sub>4</sub> each represents a hydrogen atom, an alkyl group, an aralkyl group or an aryl group, and R<sub>1</sub>, R<sub>2</sub>, R<sub>3</sub> and R<sub>4</sub> may be the same or different.

\* \* \* \* \*

UNITED STATES PATENT AND TRADEMARK OFFICE  
CERTIFICATE OF CORRECTION

PATENT NO. : 5,176,976

Page 1 of 2

DATED : January 5, 1993

INVENTOR(S) : TOSHIHIRO KIKUCHI, ET AL.

It is certified that error appears in the above-identified patent and that said Letters Patent is hereby corrected as shown below:

COLUMN 1

Line 7, "Invent" should read --Invention--.

Line 23, "an" should read --and--.

Line 40, "publication" should read --Publication--.

Line 61, "bad" should be deleted, (second occurrence).

COLUMN 2

Line 40, "Organic" should read --organic--.

Line 46, "and," should read --and--.

COLUMN 3

Line 18, "different one" should read --different--.

Line 19, "another." should be deleted.

COLUMN 4

Line 25, Under Exemplary Compound (7),

"R<sub>1</sub>, R<sub>2</sub>: H" should read --R<sub>1</sub>, R<sub>2</sub>:-H--.

COLUMN 5

Line 61, "oases" should read --cases--.

Line 68, "the" should read --of the--.

COLUMN 10

Line 16, "in" should read --in the--.

Line 18, "their" should read --the--.

Line 20, "the" (second occurrence) should be deleted.

--

UNITED STATES PATENT AND TRADEMARK OFFICE  
CERTIFICATE OF CORRECTION

PATENT NO. : 5,176,976

Page 2 of 2

DATED : January 5, 1993

INVENTOR(S) : TOSHIHIRO KIKUCHI, ET AL.

It is certified that error appears in the above-identified patent and that said Letters Patent is hereby corrected as shown below:

COLUMN 12

Line 23, "nd" should read --and--.

Line 30, "alcohol soluble" should read --alcohol-soluble--.

COLUMN 14

Line 36, "1.6 hours" should read --1.5 hours--.

COLUMN 17

Line 49, "CHARGING" should read --charging-- and  
"DE-" should read --a developing--.

Line 50, "VELOPING" should be deleted.

COLUMN 18

Line 21, "member, developing" should read --member,  
charging means, developing--.

Signed and Sealed this

Thirtieth Day of November, 1993

Attest:



BRUCE LEHMAN

Attesting Officer

Commissioner of Patents and Trademarks

--